

## UNITED STATES PATENT OFFICE

2,089,192

## MANUFACTURE OF TEXTILE THREADS AND FABRICS

Henry Dreyfus, London, England

No Drawing. Application March 14, 1935, Serial No. 11,078. In Great Britain March 21, 1934

## 9 Claims. (Cl. 117—2)

This invention relates to the manufacture of crêpe threads of cellulose acetate or other cellulose ester or ether, and to the production of fabrics therefrom.

- 5 In the past, great difficulty has been experienced in producing, with the aid of cellulose ester or ether threads to which a crêpe twist has been imparted, fabrics exhibiting crêpe effects of the kind readily obtainable by weaving a fabric from 10 highly twisted yarns of natural silk in the gummed state and subjecting the fabric to a hot aqueous treatment. Generally, substantially no crêpe effect is obtainable by simply applying to cellulose acetate thread a twist of the order of 15 that commonly employed in connection with natural silk crêpe threads, weaving the twisted threads into a fabric and subjecting the latter to a hot aqueous treatment.

In accordance with the present invention in applying a crêpe twist to threads of cellulose acetate or other cellulose esters or ethers at least the last part of the crêpe twist is applied whilst the material of the thread is in a softened state. In this way it is possible to produce cellulose acetate or other cellulose ester or ether crêpe threads having, as compared with threads produced by a simple twisting operation, greatly improved properties, particularly as regards strength and the ability to yield fabrics exhibiting good crêpe effects.

The softening of the material of the threads may advantageously be effected by subjecting the threads to the action of softening agencies during the actual application of crêpe twist. Thus 25 the thread may be twisted on a device of the kind in which the thread is drawn off over the end of a rotating package and allowed to pass, on its way to a winding device, through a body of a liquid softening agent.

- 40 The agencies contemplated for use in accordance with the present invention are more particularly those which have a mild softening or plasticizing effect on the material of the filaments, and particularly such agencies the softening effect of which may rapidly and completely be dispelled when they have served their purpose. As examples of agents which may be employed to effect the desired temporary softening or plasticizing of the filaments in accordance with the 45 present invention, mention may be made of those organic liquids which have a mild softening action on cellulose esters or ethers, particularly a softening action of the order of that of boiling water on cellulose acetate. Volatile organic liquids are 50 convenient in that materials softened by them

may quickly and easily be restored to their original condition by volatilization of the liquid. In the case of treating cellulose esters, mention may be made of the following as examples of liquids which may be used to effect the softening of the 5 cellulose ester:—aliphatic hydrocarbons, for example low-boiling fractions of petroleum, or aromatic hydrocarbons, for example benzene, toluene, xylenes, or mixtures of these hydrocarbons; aliphatic alcohols for example methyl or 10 ethyl alcohol, or higher alcohols, e. g. propyl, butyl or amyl alcohols, or glycol, glycerol or other di- or poly-hydric alcohols; ethers, for example dialkyl ethers, e. g. di-isopropyl ether and mono-, di-, or poly-ethers of glycol, glycerol or other di- or poly-hydric alcohols. Again, esters may be used e. g. ethyl acetate, ethyl lactate, or ethyl-oxy-butyrate. Substances of high swelling or solvent action on the material of the threads may be diluted with substances of low swelling 20 action, e. g. hydrocarbons.

Instead of employing organic liquids as softening agents, aqueous liquids containing substances which impart to the aqueous liquid a softening or swelling action on cellulose esters or 25 ethers, may be employed. Thus, aqueous solutions of organic solvents or swelling agents for cellulose esters or ethers may be used, the concentration of the organic substance being adjusted according to the precise degree of softening power 30 required. For example, aqueous solutions of phenol, acetone, pyridine, alcohol, glycol, ethers or esters of glycol, e. g. mono-ethyl-ether of ethylene glycol, may be used. Again, aqueous solutions of inorganic agents having a solvent or 35 swelling action on cellulose esters or ethers may be employed, for example aqueous solutions of thiocyanates.

The aqueous or other liquids employed may be 40 used either hot or cold, according to their softening action on the cellulose esters or ethers, and according to the precise degree of softening required. In general, it is advantageous to employ liquids having the desired softening or plasticizing 45 action when hot, but little or no softening or plasticizing action when cold, e. g. glycol or glycerol. By the use of such liquids the desired transient softening of the material of the filaments may readily be secured.

The liquid softening agent may be employed under pressure, for example pressures of a few pounds per square inch or pressures of several atmospheres.

Liquid aqueous softening agents may contain 55

substances which facilitate wetting of the threads by the liquid.

Still another method of effecting the desired temporary softening or plasticizing of the material of the filaments is to utilize the vapors of organic substances and especially of such organic substances as do not have a strong solvent or softening action on the materials. The vapors may be saturated or superheated or employed 10 in the presence of the substance in liquid form. As examples of suitable vapors may be mentioned those of aliphatic alcohols, e. g. methyl, ethyl, propyl, butyl or amyl alcohol, and those of aliphatic or aromatic hydrocarbons or of certain 15 halogenated organic compounds, for example carbon tetrachloride, or mixtures thereof. The vapors may be employed at atmospheric pressure or at pressures below or above atmospheric pressure, for example at 5 to 20 lbs. per square inch 20 or more above atmospheric pressure.

Steam may be used in conjunction with the softening agents if desired. Thus threads containing or moistened with softening agents may be subjected to the action of steam during twisting. Again, softening may be effected with the aid of a mixture of steam and the vapor of an 25 organic softening agent.

If desired, the requisite softening of the material of the filaments may be effected by means 30 of heat and without the use of a substance which itself has a softening action on the material of the filaments. Thus, the softening may be effected by means of a heated gas, or by means of a superheated vapor.

35 In carrying out the new process, twisting is most advantageously effected on a device of the kind in which the thread is drawn off over the end of a rotating package through a guide fixed substantially in line with the axis of rotation of the package and is thereafter wound on a bobbin or the like, the thread being softened on its way from the guide to the bobbin. In this way the thread is in a softened state during the actual application of twist.

45 On the other hand, any other suitable crêpe twisting device may be employed. For example a ring twister may be used.

The twisting spindle, the guide fixed in line with the axis of the spindle, and the means for 50 softening the thread, should be so arranged that the twist resulting from the rotation of the package is at least partly inserted while the thread is in a softened state. If the freedom of the thread to rotate within the balloon guide or 55 other guide preceding or forming part of the liquid treatment device is unduly restricted, e. g. by causing the thread to change direction materially at the guides, the insertion of twist while the thread is in a softened state may be restricted 60 to an undesirable extent or substantially prevented and the resulting crêpe threads may not have the valuable properties which may otherwise be secured. Using a twisting device of the kind in which thread is drawn off over the end 65 of a rotating package, it is advantageous to arrange that the path of the thread after leaving the balloon guide and through the zone in which softening is effected, is substantially in line with the axis of the spindle.

70 If desired, the above-mentioned twisting devices, in which the thread is drawn off over the end of a rotating package, may be provided with a device which restricts the ballooning of the thread or the tendency of twist to run back to the package. As examples of such devices may be men-

tioned flyers and the floating ring device described in U. S. Patent No. 1,784,581. The latter device is of particular value when the thread to be twisted is of very low twist, for example less than about 1 turn per inch.

5 The treatment of the thread with a liquid softening agent during twisting may be effected by drawing the thread off from a twisting spindle and passing it upwardly through a small hole in a suitable receptacle containing the liquid, the 10 thread then passing to a winding device. The hole may be, for example, about  $\frac{1}{4}$  of an inch in diameter and may be provided with means adapted to lead away and prevent from reaching the twisting spindle, any liquid issuing from the hole. 15 If desired, the hole may take the form of a short tube of fine bore, fixed in the receptacle, whereby the flow of liquid from the receptacle at the point of entrance of the thread may be reduced. Another method is to supply the liquid to the thread. 20 For example, the thread may be caused to pass in contact with a wick dipping into the liquid or in contact with a horizontally disposed roller, preferably circumferentially grooved, arranged to rotate in a bath of the liquid and so to carry it to the thread. In the case of using hot liquids the liquid may be supplied to the thread in a heated state or it may be applied to the thread at a lower 25 temperature and the thread then heated, e. g. by passing it through a heated chamber on its way to the winding device.

30 The zone in which the thread is in a softened state may be relatively short, for example 1 to 3 inches.

35 In the case of using vapors to effect the desired softening the thread may be drawn off from a twisting spindle and passed through a suitable chamber supplied with the particular vapor in question.

40 Thus, a vertical twisting spindle of the type in which thread is drawn off upwardly over the end of a rotating package through a guide substantially in line with the axis of the spindle, may be provided with a small chamber situated vertically above the spindle. The chamber is provided 45 with small holes, top and bottom, to permit passage of the thread, and also with a vapor inlet. If desired, a single vapor chamber may be arranged to serve a number of spindles, being provided with inlet and outlet holes for the thread 50 of each spindle. Such an apparatus may conveniently consist of a horizontal pipe mounted over a row of spindles and provided with eyes of porcelain, stainless steel, or other suitable material at appropriate points on top and bottom for the entrance and exit of the threads. The diameter of the pipe is sufficient to afford the thread 55 the requisite length of travel in the vapor. Vapor may be admitted to the pipe at one point or at more than one point as may be necessary according to the length of the pipe, to secure sufficiently uniform conditions of steaming as between the threads from the different spindles.

60 If desired vapors of the softening agents may be employed in the presence of a liquid softening agent. The presence of liquid softening agent 65 may be assured by arranging for condensation of the vapor in the vapor treating device. Another method of ensuring the presence of liquid softening agent is to moisten the thread therewith; for example the liquid may be applied to the thread by means of a wick or other device after the thread leaves the spindle and prior to its entering the vapor treatment device.

70 If desired a softening agent may be incorporat-

ed in the threads in an operation separate from the crêpe twisting operation. Thus, packages of threads may be impregnated with an appropriate softening agent and thereafter crêpe twisted. For example, the threads in package form may be subjected to the action of vapor of a solvent or they may be dipped into a liquid softening agent. Softening agents of high boiling point may be applied in solution in a volatile liquid, e. g. benzene or petrol, and if desired the latter removed by evaporation. In the case of volatile softening agents it is preferable, in order to avoid loss of volatile softening agent, to twist on a device of the kind in which the thread is drawn off from a stationary or slowly rotating package and twisted as it is wound on to a second package.

Again, if desired, cellulose ester and ether threads may be twisted immediately after their formation by dry or wet spinning methods and while they still contain a solvent or a constituent of a spinning bath of such nature and in such proportion as to afford the desired degree of softness. For example, cellulose acetate threads containing 8-25%, e. g. 10-20%, of acetone may be twisted. Threads containing other solvents may be used, e. g. threads containing dichloroethylene and alcohol, benzene and acetone, or alcohol and acetone. In the case of producing threads containing softening agents by dry spinning processes high boiling softening agents or plasticizers, e. g. diethyl phthalate, dibutyl phthalate, triacetin, etc., may be incorporated in the spinning solution, and/or spinning effected at comparatively low temperatures in order to leave the desired proportion of softening agent in the filaments. Again, there may be added to the spinning solution substances which retard the evaporation of solvent. Cetyl alcohol and other alcohols, for example in amounts of 10-20% of the weight of the cellulose ester or ether may be used for this purpose.

The initial thread may already be twisted to a small degree, for example up to 10 turns per inch, e. g. to 2 to 5 turns per inch or to such small degree as is commonly applied in the production of cellulose acetate threads by dry spinning cellulose acetate solutions and winding and twisting the resultant filaments on a cap twisting device.

In carrying out the new process the crêpe twist may be applied in a single stage. If desired, however, the twist may be applied in two or more stages, the final stage of twisting being effected whilst the material of the thread is in a softened state.

When the crêpe twist is applied in two or more stages the advantages of the process may be obtained when not only the final stage of the crêpe twisting but an earlier stage or stages of twisting are also effected whilst the material of the thread is in a softened state. In fact it is of great advantage to effect, while the material of the thread is in a softened state, any application of twist beyond the point at which twisting would result in weakening of the thread if the said twisting were effected while the material of the thread was not in the softened state.

The precise degree of twist beyond which it is important that the material of the thread should be in a softened state during twisting depends upon the total denier of the thread and the number of its constituent filaments. Generally at least the last two-thirds of the total crêpe twist should be applied whilst the material of the thread is in a softened state.

The cellulose ester or ether filaments of the

threads very readily undergo stretching when the threads are twisted while in a softened state. The amount of stretch may be measured by comparing the original thread denier with the final thread denier (after untwisting). It has been found that when a cellulose ester or ether thread is crêpe twisted while in a softened state so as to produce a crêpe thread of good strength and crêping properties, the denier of the resultant thread is, in general, owing to imparted stretch, less and even substantially less than if the thread is simply crêpe twisted in the ordinary manner. The stretch imparted to the filaments of the threads during the twisting operation may for example be of the order of 5-25% of their original length, and particularly 10-20%. The degree of stretching of the filaments of the thread may be such that the final denier of the crêpe twisted thread is not much in excess of or is even the same or less than the denier of the thread prior to twisting. For example the stretch may be such that the denier of the crêpe twisted thread is from 95 to 115%, particularly 100 to 110% of that of the thread before crêpe twisting, especially in the case of threads having an original denier of 150 or less. Good crêpe fabrics may however be obtained when the final denier is still greater, for example up to 120% of that of the thread before twisting when threads having a denier about 200 are employed.

The degree of twist applied in accordance with the new process may vary within wide limits. A feature of the process is that it enables a high degree of twist to be applied without such a great weakening of the thread as is almost invariably experienced when cellulose ester or ether crêpe threads are prepared by ordinary methods of crêpe twisting. The process, moreover, permits the insertion of twists which are impossible of attainment when the thread is not in the softened state. This is important since it enables crêpe fabrics to be produced having very pronounced crêpe effects. The crêpe figure can be regulated according to requirements. The degree of twist desirable in any particular case depends upon the denier of the thread. For example with threads of 165 denier twist of about 70 to 75 turns per inch is desirable, and with threads of 115 denier twist of about 85 to 90 turns per inch. With these indications it is a simple matter to determine the desirable twists for threads of other deniers. The denier numbers given are those of the threads after crêpe twisting.

As indicated above, the new process enables highly twisted cellulose ester or ether threads of of high crêping power to be produced. In these new threads the filaments are extremely closely packed, a feature to which their good crêping power may be attributed. For example, the filaments may be so closely packed that the apparent specific gravity of the thread as determined from the diameter and denier is more than 85%, e. g. 85 to 90% of the actual specific gravity of the filaments, and that distortion of the cross-section of at least some of the filaments has occurred during the process of twisting. The filaments of the thread, however, are not stuck together and can be separated upon untwisting. Moreover, the new cellulose ester or ether crêpe threads are smooth and cylindrical as opposed to the rough feel and helical form of a cellulose ester or ether thread or a viscose thread which has been crêpe twisted in the ordinary way. Further, in comparison with these latter threads, the smooth cylindrical cellulose ester or ether crêpe threads

exhibit much less tendency to snarl or kink. These characteristics distinguish the new cellulose ester or ether crêpe threads.

The invention is of particular value in connection with the production of crêpe threads of filaments of cellulose acetate. Crêpe threads of filaments of other cellulose esters or cellulose ethers may, however, be produced by the new method.

As examples of cellulose esters of which the filaments of the crêpe threads may be made, mention may be made of nitrocellulose or of organic esters of cellulose, for example cellulose formate, cellulose propionate or cellulose butyrate. If desired, the filaments may be made of mixed esters of cellulose, for example cellulose nitroacetate or cellulose acetate-butyrate. Methyl cellulose, ethyl cellulose and benzyl cellulose are examples of cellulose ethers of which the threads may be made. Again, if desired, filaments made of ether-esters of cellulose may be employed, for example filaments of a low ether cellulose which has been acetylated or otherwise esterified, or filaments of an esterified (hydroxy-alkyl)-ether of cellulose, e. g. acetylated (hydroxy-ethyl)-cellulose.

The crêpe threads may be made with filaments such as have been prepared by extruding into a coagulating medium a solution of the cellulose ester or ether in a suitable solvent. Again, they may be such as have been prepared by esterification of cellulose filaments without losing the filamentary form of the latter, e. g. filaments of regenerated cellulose which have been esterified by means of acetic anhydride, butyric anhydride or other esterifying agent.

The threads may contain substantially continuous filaments of cellulose esters or ethers or they may contain discontinuous filaments of the esters or ethers, the length of which may vary within wide limits. For example the threads may be those spun from a mass of discontinuous filaments or those prepared in the manner described in British Patents Nos. 424,683, 424,752, 424,830 and 424,879.

If desired there may be employed threads consisting of or containing cellulose ester filaments which have been superficially saponified or have been partially saponified throughout. The saponification may be effected intermittently along the length of the threads.

The invention is of particular advantage in connection with the production of crêpe threads consisting wholly of cellulose acetate or other cellulose ester or ether filaments. If desired, however, the threads may be composed in part of filaments of one ester or ether of cellulose and in part of filaments of another ester or ether of cellulose, or in part of filaments of a cellulose ester or ether and in part of filaments of another material, for example natural silk or regenerated cellulose. As in the case of the cellulose ester or ether filaments, such other filaments may be substantially continuous filaments and/or discontinuous filaments.

While the new process enables production of threads which yield satisfactory crêpe effects without a special treatment, other than the twisting and softening treatment characteristic of the process, other devices and treatment may, if desired, be employed further to improve the properties of the crêpe threads and/or fabrics produced therefrom. For example, the twist may be irregular in character as described in British Patent No. 385,585. Further, the crêpe threads may be sized, uniformly or intermittently along their length at any suitable stage of

their manufacture, for example prior to the application of twist, or at least any substantial proportion of the twist. In this connection, particular mention may be made of sizing materials selected in accordance with the considerations laid down in U. S. Patent No. 2,007,182. For example a casein, egg-albumen or other size which is not very readily removed by aqueous treatments may be employed. Another size which may be employed is a drying oil, if desired one which has been partially oxidized, e. g. boiled or blown linseed oil. Hygroscopic substances, for example sodium acetate, calcium chloride, calcium nitrate, citric acid, glycerine, sodium lactate etc., may be incorporated in the materials prior to the crêpe twisting, for example, in the case of threads of extruded filaments, by way of the spinning solutions from which the threads are prepared. In such a case the threads may already contain sufficient moisture to give the desired softening so that either at ordinary temperatures or at suitably raised temperatures, produced for example by the simple application of hot air, dry steam or the like, the improved crêpe twisting is obtained.

Another treatment which is sometimes found beneficial is a wetting treatment. Such wetting may be effected, for instance, before or during the application of the crêpe twist. Thus, the thread may be wetted as it leaves a twisting spindle, and prior to passage through a vapor or hot gas treatment device.

The highly twisted crêpe threads may be incorporated in the fabrics in various ways, for example the weft alone may be wholly or partially composed of such threads or the warp may also contain them. Valuable fabrics may be produced by employing warp threads of relatively low twist and in the weft both crêpe threads having a left-hand twist and crêpe threads having a right-hand twist, pairs of threads of left-hand twist alternating with pairs of threads of right-hand twist.

Fabrics containing highly twisted crêpe threads prepared in accordance with the invention may subsequently be subjected to a hot aqueous treatment, for example in the manner commonly adopted in connection with fabrics comprising highly twisted crêpe threads of natural silk. Such treatment may be, for instance, a treatment in an aqueous soap bath at a temperature of 75-85° C. or at higher temperatures, e. g. at the boil. If desired the fabrics or the threads from which they are prepared may be treated, prior to the hot aqueous treatment, so as to remove wholly or in part any softening agent, such removal may be effected for example by heating or by washing with a suitable liquid, e. g. benzene.

Fabrics containing highly twisted threads prepared in accordance with the invention may also be subjected to a treatment adapted to swell the material of the filaments of the said threads. Such treatment may be in addition to the hot aqueous treatment of the woven fabric, and may be effected before or after, or simultaneously with, the said hot aqueous treatments.

The term "organic derivative of cellulose" used in the appendant claims connotes a cellulose ester of an organic acid or a cellulose ether.

What I claim and desire to secure by Letters Patent is:—

1. Process for the production of highly twisted cellulose acetate crepe threads, which comprises crepe twisting cellulose acetate threads and, dur-

5 ing the insertion of at least the last part of the crepe twist, treating the threads with an organic softening agent therefor so that during twisting the filaments of the threads are so softened and stretched that the final thread denier is less than 115% of that of the thread before crepe twisting.

2. Process for the production of highly twisted cellulose acetate crepe threads, which comprises crepe twisting cellulose acetate threads which, 10 during the insertion of at least the last part of the crepe twist, are so soft under the action of an organic softening agent that during twisting the filaments of the threads become so closely packed together that the apparent specific gravity of the 15 threads is at least 85% of that of the material of the filaments.

3. Process for the production of highly twisted cellulose acetate crepe threads, which comprises applying to a cellulose acetate thread a minimum 20 crepe twist determined according to the denier, the said minimum being 70 turns per inch for thread of 165 denier and 85 turns per inch for thread of 115 denier, and softening the thread with an organic softening agent during the insertion of at least the last part of the twist so that 25 the filaments of the thread stretch so much that the denier of the final thread is less than 115% of that of the thread before twisting.

4. Process for the production of highly twisted cellulose acetate crepe threads, which comprises crepe twisting cellulose acetate threads in at least 30 two stages, and during the final stage of twisting treating the threads with an organic softening agent therefor, so that the material of the threads 35 is softened to such a degree that the filaments undergo substantial stretching during the twisting.

5. Process for the production of highly twisted cellulose acetate crepe threads, which comprises 40 crepe twisting cellulose acetate threads and, during the insertion of at least the last part of the crepe twist, treating the threads with an organic softening agent therefor so that during twisting the filaments of the threads are so softened and

stretched that the final thread denier is less than 120% of that of the thread before crepe twisting.

6. Process for the production of highly twisted cellulose acetate crepe threads, which comprises crepe twisting cellulose acetate threads and, during 5 the insertion of at least the last part of the crepe twist, treating the threads with an organic liquid softening agent therefor so that during twisting the filaments of the threads are so softened and stretched that the final thread denier 10 is less than 115% of that of the thread before crepe twisting.

7. Process for the production of highly twisted crepe threads of an organic derivative of cellulose, which comprises crepe twisting threads of an 15 organic derivative of cellulose and, during the insertion of at least the last part of the crepe twist, treating the threads with an organic softening agent therefor so that during twisting the filaments of the threads are so softened and stretched 20 that the final thread denier is less than 115% of that of the thread before crepe twisting.

8. Process for the production of highly twisted crepe threads of an organic derivative of cellulose, which comprises crepe twisting threads of an 25 organic derivative of cellulose in at least two stages, and during the final stage of twisting treating the threads with an organic softening agent therefor, so that the material of the threads 30 is softened to such a degree that the filaments undergo substantial stretching during the twisting.

9. Process for the production of highly twisted crepe threads of an organic derivative of cellulose, which comprises crepe twisting threads of an 35 organic derivative of cellulose and, during the insertion of at least the last part of the crepe twist, treating the threads with an organic softening agent therefor so that during twisting the filaments of the threads are so softened and stretched 40 that the final thread denier is less than 120% of that of the thread before crepe twisting.

HENRY DREYFUS.